# EUROPEAN PATENT APPLICATION

(11) **EP 0 777 009 A2**
(43) Date of publication of application: **04.06.1997**
(21) Application number: 96308474.4
(22) Date of filing: 22.11.1996
(51) Int. Cl.: D06M 15/643, D06M 15/65, D06M 15/277

(54) **Compositions for treating fibers and textiles**

(30) Priority: 28.11.1995 JP 334050/95
(71) Applicant: Dow Corning Toray Silicone Company Ltd., Tokyo (JP)
(72) Inventor: Ishikawa, Hiroki, Dow Corning Toray, Ichihara-shi, Chiba Pref. (JP); Naganawa, Tsutomu, Dow Corning Toray, Ichihara-shi, Chiba Pref. (JP); Ona, Isao, Dow Corning Toray, Ichihara-shi, Chiba Pref. (JP)
(74) Representative: Dowden, Marina

(57) **Abstract**

Compositions for treating fibers and textile are prepared from (A) a vinyl polymer having perfluoroalkyl groups with a carbon number of at least 5 and (B) organopolysiloxanes that have radicals containing one or more epoxy groups and one or more carboxyl or alkoxysilyl group derivatives.

## Description

The present invention provides compositions for treating fibers and textiles, and more specifically, to compositions that impart said fibers and textiles with superior water repellency, oil repellency and excellent hand.

Compositions for treating fibers and textiles which include a perfluoroalkyl-radical-containing vinyl polymer are known to impart the properties of water repellency and oil repellency. Furthermore, those treatment compositions which are obtained by adding and mixing organopolysiloxanes having hydroxy, epoxy, amino or carboxyl radicals to such vinyl polymers are also known from JP-B 58-1232 and 59-47071, or JP-A 60-75678.

However, the fiber and textile treatment compositions of the prior art suffer from the drawback that they achieve very poor hand and insufficient water repellency.

In the present invention, there is provided a novel composition for treating fibers and textiles, which overcomes the drawbacks of the prior art. Our fiber and textile treatment composition comprises:
(A) 100 parts by weight of vinyl polymer having perfluoroalkyl radicals with a carbon number of 5 or greater, and
(B) 5-50 parts by weight of organopolysiloxanes that have one or more epoxy-containing organic radicals, and one or more carboxyl groups represented by the formula:

   -COOR⁶

   wherein R⁶ is a monovalent radical selected from the group consisting of hydrogen atoms, hydrocarbon radicals, and silyl radicals represented by the formula:

   -SiR₃

   wherein each R is a radical independently selected from monovalent hydrocarbon radicals having 1-10 carbon atoms or radicals represented by the formula:

   -R³-SiR₃₋ₐ(OR⁴)ₐ

   wherein R is as above, R³ is selected from divalent hydrocarbon radicals or sulfur-containing divalent hydrocarbon radicals, R⁴ is selected from hydrogen atoms or monovalent hydrocarbon radicals, and a is an integer from 1 to 3.

As used herein for component (B), the term "carboxyl groups" describes those groups represented by the formula -COOR⁶, wherein R⁶, by definition, is not limited to hydrogen atom. Those skilled in the art will appreciate that the term "carboxyl groups", as used herein, includes carboxyl group derivatives which are in conformity with the general formula -COOR⁶.

It is an object of this invention to provide a novel composition for treating fibers and textiles that impart superior water repellency, oil repellency and excellent hand.

The vinyl polymers having perfluoroalkyl radicals with a carbon number of 5 or greater, component (A) of the present invention, are any compound which meets the aforesaid limitations and is conventionally used for fiber treatment. For example, homopolymers of reactive monomers having perfluoroalkyl radicals, and copolymers of these monomers with other reactive monomers that do not contain perfluoroalkyl radicals are useful. Compounds represented by the formulas below are examples of reactive monomers having perfluoroalkyl radicals.
CH₂=CHC₈F₁₇
CH₂=C(CH₃)CH₂C₁₀F₂₁
CF₃(CF₂)₉(CH₂)₂OCH=CH₂
CF₃(CF₂)₈(CH₂)₂OCOCH=CH₂
CF₃(CF₂)₇(CH₂)₁₁OCOCH=CH₂
CF₃(CF₂)₈(CH₂)₂OCOC(CH₃)=CH₂
CF₃(CF₂)₄CH₂OCOC(CH₃)=CH₂
(CF₃)₂CF(CF₂)₆(CH₂)₃OCOCH=CH₂
(CF₃)₂CF(CF₂)₁₀(CH₂)₃OCOCH=CH₂
(CF₃)₂CF(CF₂)₆(CH₂)₂OCOCH=CH₂
CF₃(CF₂)₇SO₂N(C₃H₇)(CH₂)₂OCOCH=CH₂
CF₃(CF₂)₇SO₂N(CH₃)(CH₂)₂OCOC(CH₃)=CH₂
(CF₃)₂CF(CF₂)₆CH₂CH(OH)CH₂OCOCH=CH₂
(CF₃)₂CF(CF₂)₆CH₂CH(OCOCH₃)OCOC(CH₃)=CH₂
CF₂Cl(CF₃)CF(CF₂)₇CONHCOOCH=CH₂
H(CF₂)₁₀OCOCH=CH₂
CF₂Cl(CF₂)₁₀CH₂OCOC(CH₃)=CH₂

Various compounds, such as N-methylolacrylamide, N-methylolmethacrylamide, glycidyl acrylate, glycidyl methacrylate, aziridinyl acrylate, aziridinyl methacrylate, diacetone acrylamide, diacetone methacrylamide, methylol diacetone acrylamide, methylene diacrylate, ethylene diacrylate, hydroxyalkyl acrylate, hydroxyalkyl methacrylate, 3-fluoro-2-hydroxypropyl methacrylate, are other suitable reactive monomers that do not have perfluoroalkyl radicals. Vinyl chloride, ethylene, vinyl acetate, vinyl fluoride, acrylamide, methacrylamide, styrene, a-methylstryrene, halogenated alkyl vinyl ether, benzylalkyl ether, alkyl esters of acrylic acid or methacrylic acid, benzyl alkyl ether, vinyl alkyl ketone, cyclohexyl acrylate or methacrylate, anhydrous maleic acid, butadiene, isopropylene, chloropropylene are acceptable in addition to the above. These monomers are used alone, or as a combination of two or more, for reaction with our monomers having perfluoroalkyl radicals.

Preferably, the ratio of copolymerization (wt%) of the above monomers that contain perfluoroalkyl radicals, and monomers that do not contain perfluoroalkyl radicals, is within the range of 10-90 to 90-10. More preferably, the range is from 30-80 to 70-20. This type of copolymer is formulated by subjecting the above monomers to copolymerization under solution polymerization, emulsion polymerization or some other well-known method by using radical initiators. Polymerization catalysts used for radical polymerization of vinyl resins are preferable as radical initiators. For example, benzoyl peroxide, dichlorobenzoyl peroxide, dicumyl peroxide, di-t-butyl peroxide, 1,3-bis(t-butylperoxyisopropyl)benzene, lauryl peroxide, t-butyl peracetate and other organic peroxide catalysts; azobisisobutyronitrile, dimethylazodiisobutyrate and other azo compound catalysts or redox catalysts are all useful herein.

The copolymerization reaction is conducted in the presence of acetone, methyl isobutyl ketone, methyl ethyl ketone, trichloroethylene, perchloroethylene, trifluoroethane, trichlorotrifluoroethane, toluene and other organic solvents, higher alcohol polyoxyalkylene adducts, higher fatty acid polyoxyalkylenephenol polyoxyalkylene adducts and other emulsification agents and water. It is preferable for the reaction temperature to be within the range of 30-100°C, and the reaction time to be within 1-30 minutes.

Component (B) of our invention, includes organopolysiloxanes having one or more epoxy-radical-containing organic radicals and one or more radicals represented by the above formulas and organic radicals containing epoxy radicals. This component, and its aforementioned radicals, surprisingly function to improve the hand imparted to fibers and textiles treated therewith, and they also resist removal during laundering. Organopolysiloxanes represented by the following general formula are suitable for use as component (B) in the present invention:

In the above formula (I), each R is a radical independently selected from monovalent hydrocarbon radicals having 1 - 10 carbon atoms. More specifically, the R groups are preferably methyl, ethyl, propyl, octyl and other alkyl radicals; 2-phenylethyl radicals, 2-phenylpropyl radicals, 3,3,3-tolufluoropropyl; 3,3,3-trifluoropropyl radicals or halogen substituted alkyl radicals; phenyl radicals, tolyl radicals and other aryl radicals or substituted aryl radicals. Among them, methyl radicals are most preferred.

Also in formula (I) B* is an organic radical containing an epoxy radical represented by or an organic radical containing an epoxy radical represented by wherein R¹ and R² are divalent hydrocarbon radicals, such as ethylene, n-propylene, isopropylene, and n-butylene.

Also in formula (I), C* is a radical represented by the formula

(II) -R³-SiR₃₋ₐ(OR⁴)ₐ

or a carboxyl radical represented by the formula

(III) -R⁵-COOR⁶.

In these formulas, (II) and (III), R³ and R⁵ are divalent hydrocarbon radicals or sulfur-containing divalent hydrocarbon radicals.

Specifically, ethylene radicals, n-propylene radicals, n-butylene radicals and other alkylene radicals or alkylene arylene radicals represented by the formula

-(CH₂)₂-C₆H₄-

are examples of suitable divalent hydrocarbon radicals.

Groups represented by the formula

-CH₂-S-CH₂CH₂-S-

and radicals represented by the formula

-CH₂CH₂-S-CH₂-

are examples of sulfur-containing divalent hydrocarbon radicals.

In formula (II), R⁴ is a hydrogen atom or a monovalent hydrocarbon radical, with methyl and ethyl radicals being preferable as the monovalent hydrocarbon radicals. The subscript a is a positive number from 1-3.

In formula (III), R⁶ is a radical selected from the group consisting cf hydrogen atoms, monovalent hydrocarbon radicals and silyl radicals represented by the formula -SiR₃, wherein R is as defined above.

In formula (I), A* is a radical selected from the group consisting of R, B* and C*. The subscript x is a positive number, y is 0 or a positive number and z is 0 or a positive number. There are no particular limitations concerning the value of (x + y + z), but it is preferable for it to be within the range of 50-1,000. When it is less than 50, the hand of the fibers or textiles after treatment is insufficient. When it exceeds 1,000, there is a decrease in handling properties, productivity, and emulsification properties. It is preferable for the content of epoxy-radical-containing organic radicals, carboxyl groups and groups represented by the formula -R³-SiR₃₋ₐ(OR⁴)ₐ in these diorganopolysiloxanes to be within the range of 0.5-3 mole% of all the organic radicals that are bonded to silicon atoms.

The diorganopolysiloxanes represented by general formula (I) are manufactured by the following methods.

For example, the following ingredients may be simultaneously reacted:
an organic compound represented by the formula

   CH₂=CH(CH₂)₈COOSi(CH₃)₃
an epoxy-radical-containing organic compound represented by the formula
and a diorganopolysiloxane having a hydrogen atom in the side chain, represented by the formula

   (CH₃)₃SiO[(CH₃)₂SiO]ₓ[(CH₃)HSiO]_{y}Si(CH₃)₃
wherein x is a positive number and y is a positive number, as above;
in the presence of 10-20 ppm of an addition reaction catalyst such as platinum chloride.

By adding a small amount of alcohol or a mixture of alcohol with water, the trimethylsilyl radicals are converted to hydrogen atoms; thus, obtaining diorganopolysiloxanes represented by the following formula: wherein b + c = y.

In this formula, siloxane units that have epoxy-radical-containing organic radicals, and siloxane units that have carboxyl radicals, are bonded in a random fashion.

In like manner, diorganopolysiloxanes represented by the formula wherein b + c = y. In this latter formula, siloxane units that have epoxy-radical-containing organic radicals, and siloxane units that have alkoxysilyl radicals, are bonded in a random fashion. These are obtained by using an alkoxy-containing organic compound represented by the formula CH₂=CHSi(OCH₃)₃ instead of using an organic compound represented by the formula CH₂=CH(CH₂)₈COOSi(CH₃)₃.

Compounds represented by the formulas below are also examples of the organopolysiloxanes of component (B).

The amount of component (B) that is added to component (A) is within the range of 5-50 parts by weight, and preferably is, 20-40 parts by weight, per 100 parts by weight of component (A). If less than 5 parts by weight of (B) are used, the composition fails to impart the fiber or textile with good hand. If more than 50 parts by weight of (B) are used, then there is a marked decrease in water and oil repellency, in particular, oil repellency.

The composition of this invention is a composition made up of the above-mentioned components (A) and (B). However, antistatic agents, dye stabilizing agents, anticrease agents, antiseptics, antimildew agents, rust-preventing agents as well as organic solvents such as toluene, xylene, hexane, heptane, perchloroethylene, 1,1,1-trichloroethane and the like can be added and mixed therewith, as long as they do not defeat the desirable properties imparted by our composition to fibers and textiles.

The composition of the present invention is manufactured by means of uniformly mixing components (A) and (B). When mixing is performed, the organopolysiloxanes of component (B) are first either diluted with toluene, xylene, hexane, heptane, perchloroethylene, 1,1,1-trichloroethane or other aromatic organic solvents, aliphatic organic solvent or chlorine organic solvent, or emulsified with water and nonionic surfactants, anionic surfactants, or both. Thereafter, component (A) is added thereto. Polyoxyalkylene alkyl ethers, polyoxyalkylene alkyl esters, polyoxyalkylene sorbitan alkyl esters, sorbitan alkyl esters, polyethylene glycols, polypropylene glycols and the like are examples of nonionic surfactants that can be used. Octylbenzenesulfonic acid and other alkylbenzenesulfonic acids, higher alcohol sulfuric acid esters, polyoxyalkylene alkyl ether sulfuric acid esters, alkylnaphthylsulfonic acid sodium salt, potassium salt, lithium salt or ammonium salt are examples of anionic surfactants. The amount in which the surfactants are compounded is within the range of 3-20 parts by weight, per 100 parts by weight of organopolysiloxanes of component (B), and is preferably, within the range of 6-10 parts by weight. Emulsification is conducted under ordinary methods by using a homomixer, line mixer, colloid mill, homogenizer, Hobart^{TM} mixer, comb mixer, vacuum emulsification devices and other kneading equipment.

Generally speaking, the method of treating fibers and textiles by the composition of our claimed invention comprises soaking the fibers or textile in said composition; controlling the amount of composition adhered to the fibers or textile by squeezing, for instance by passing through a pair of rollers, and thereafter drying and subjecting the fibers or textile to heat treatment in a drier at a temperature of 120-150°C. The amount of composition which adheres depends on the type of fiber or textile. In general, however, it is preferable for the amount to be such that the total amount of component (A) and component (B), with respect to the fibers or textile, is within the range of 0.01-10.0 wt%. Fur, wool, silk, hemp, wood fiber, angora, mohair, asbestos, and other natural fibers; rayon, Bemberg^{TM}, and other regenerated fibers; acetate and other semisynthetic fibers; polyester polyamide, polyacrylonitrile, polyvinyl chloride, vinyon, polyethylene, polypropylene, spandex and other synthetic fibers; glass fiber, carbon fiber, silicon carbide fibers and other inorganic fibers are all examples of fiber materials and woven or nonwoven textiles treatable herein.

The composition of the present invention imparts superior water repellency, oil repellency and excellent hand to fibers and textiles treated therewith. Furthermore, our composition has a high affinity for fibers. For this reason, our invention has the advantage that it is superior in terms of resistance to laundering, and that the fibers after treatment maintain superior water repellency, oil repellency and excellent hand for long periods of time.

### Application Examples

Next, the present invention is explained in detail by referring to application examples. In these examples, "parts" means "parts by weight," and viscosity is a value obtained at a temperature of 25°C. In addition, the hand, oil repellency and water repellency of the fibers treated by using our fiber treatment composition were measured by the test methods described below.

### Hand

Hand was measured based on finger tactile sensation, and was evaluated in the following manner.
- A: Extremely good
- B: Good
- C: Somewhat unsatisfactory
- D: Bad

### Oil repellency

Oil repellency tests were conducted by the procedure of AATCC Test Method 118-1983. Namely, designated standard reagents, shown in Table I, were added dropwise in the amount of 0.05 mL starting from the lower grades, and the wetting of the fiber surface was observed 30 seconds later (to see how the drops permeate the fiber). Then, the highest grade among the standard reagents that did not wet the surface of the fiber was used as the grade of oil repellency.

**Table I**

| Grade | Standard Reagents |
|---|---|
| 1 | Liquid Parafin |
| 2 | A mixture of liquid paraffin and n-hexadecane [liquid paraffin:n-hexadecane = 63:35 (volumetric ratio)] |
| 3 | n-Hexadecane |
| 4 | n-Tetradecane |
| 5 | n-Dodecane |
| 6 | n-Decane |
| 7 | n-Octane |
| 8 | n-Heptane |

### Water repellency

Water repellency tests were conducted based on the method conforming to JIS L 1092 (spraying method), and measured by the standards shown in Table II.

**Table II**

| Water Repellency Grades | State |
|---|---|
| 100 | No wetting of surface was noticed |
| 90 | Slight wetting of surface was noticed |
| 80 | Water-drop wetting of the surface |
| 70 | Considerable portion of the surface was wet |
| 50 | The entire surface was wet |
| 0 | Both the front and reverse faces were completely wet |

### Application Example 1

75 parts of reactive monomer, having perfluoroalkyl groups represented by the formula CH₂=CHC₈F₁₇, and 25 parts of ethyl acrylate were dissolved in 400 parts of a methyl ethyl ketone/toluene mixed solvent (weight ratio 1:1). The solution was heated to 75°C, and 0.4 part of azobisisobutyronitrile was added thereto, whereupon the solution was kept at a temperature of 75°C for 2 h and solution polymerization was conducted. The resulting solution of copolymer had a concentration of 20%.

One part of each of the four kinds of diorganopolysiloxanes (a)-(d) was added to 15 parts of this copolymer solution, and the mixture was dissolved in 984 parts of toluene. Thus, four kinds of fiber and textile treatment compositions were prepared. Three 25 cm x 25 cm pieces of 100% cotton fabric were coated with these compositions (manufactured by Test Fabrics Inc., USA, Inter Lock Knit™). Next, these pieces of fabric were squeezed using squeezing rollers, to a squeezing ratio of 100% after which they were kept overnight at a temperature of 25°C. A squeezing ratio is defined as the weight of the textile treatment composition adhering to the fabric, divided by the weight of the fabric, expressed as a percent. Accordingly, at a squeezing ratio of 100%, the weight of the textile treatment composition adhering to the fabric is equal to the weight of the fabric. The following day, they were heat treated for 3 minutes in a hot air drier at a temperature of 150°C. The hand, oil repellency and water repellency of the fabric obtained were measured, and the results are listed in Table III. It is evident from these results that the fabric treated with our fiber treatment compositions had superior water repellency, oil repellency and hand. Thus, the claimed compositions are useful as fiber and textile treatment agents.

In addition, the chemical structures of the four kinds of diorganopolysiloxanes (a)-(d) were used as follows.

### Diorganopolysiloxane (a) :

### Diorganopolysiloxane (b):

### Diorganopolysiloxane (c) :

### Diorganopolysiloxane (d) :

### Comparative Example 1

Fiber treatment agent compositions were prepared in the same manner as in Application Example 1 with the exception of using diorganopolysiloxanes (e)-(h), represented by the formulas below, instead of using the diorganopolysiloxanes (a)-(d). 100% cotton fabric, as above, was treated with these compositions. The hand, oil repellency and water repellency of the fabric after treatment were measured, and the results are listed in Table III.

The chemical structures of the diorganopolysiloxanes (e)-(h) were as follows:

### Diorganopolysiloxane (e) :

### Diorganopolysiloxane (f) :

### Diorganopolysiloxane (g) :

### Diorganopolysiloxane (h) :

### Comparative Example 2

Textile and fiber treatment compositions were prepared in the same manner as in Application Example 1, except that no diorganopolysiloxane (B) was included in the formulations. 100% cotton fabric, as above, was treated with these compositions. The hand, oil repellency and water repellency of the fabric after treatment were measured in the manner previously described, and the results are listed in Table III.

**Table III**

| | Hand | Oil Repellency | Water Repellency | Overall Evaluation |
|---|---|---|---|---|
| Application Example 1: diorganopolysiloxanes | | | | |
| (a) | A | 4 | 90 | Extremely Good |
| (b) | A | 4 | 90 | Extremely Good |
| (c) | A | 4 | 90 | Extremely Good |
| (d) | A-B | 4 | 90 | Extremely Good |
| Comparative Example 1: diorganopolysiloxanes | | | | |
| (e) | C-B | 4 | 90 | Somewhat Insufficient |
| (f) | C | 3 | 90 | Insufficient |
| (g) | C | 3 | 80 | Insufficient |
| (h) | D-C | 2 | 80 | No good |
| Comparative Example 2: diorganopolysiloxane not added | D | 4 | 90 | No good |
| No treatment | D | 0 | 0 | ---- |

### Application Example 2

80 parts of reactive monomer having perfluoroalkyl groups, represented by the formula CF₃(CF₂)₉CH₂CH₂OCH=CH₂, 15 parts of ethyl acrylate and 5 parts of diacetone acrylamide were emulsified in an emulsifier by adding 10 parts of nonionic surfactant, represented by the formula C₁₂H₂₅O(C₂H₄O)₂₁H, and 390 parts of water. The solution was heated to 62°C and 1 part of ammonium persulfate was added thereto, whereupon the solution was kept at a temperature of 62°C for 2 h and emulsion polymerization conducted. A solution was thus prepared, wherein the concentration of the polymer obtained by the copolymerization of the monomers was 20%.

400 parts of each of the four kinds of diorganopolysiloxanes (a)-(d) of Application Example 1 were added to 35 parts of a 1:1:1 (weight ratio) mixture of three types of nonionic surfactants represented by the formulas C₁₃H₂₇(-CH₂CH₂O)₅H, C₁₃H₂₇(CH₂CH₂O)₁₂H, and C₁₃H₂₇(CH₂CH₂O)₂₁H, and 565 parts of water, and emulsification was conducted by using a comb mixer (rotation speed 2000 rpm), obtaining an emulsion with a 40% concentration.

Fiber and textile treatment compositions were prepared by diluting 30 parts of these copolymer emulsions and 5 parts of organopolysiloxane emulsions with 1965 parts of water. 100% cotton fabric pieces were soaked in the fiber treatment agent compositions obtained. Next, these pieces of fabric were after which they were kept overnight at a temperature of 25°C. The following day, they were heat treated for 3 minutes in a hot air drier at a temperature of 150°C. The hand, oil repellency and water repellency of the fabric obtained were measured, and the results are listed in Table IV. It is evident from these results that the compositions of the present invention, in the emulsified state, will impart superior water repellency, oil repellency and good hand to fiber and textiles treated therewith.

### Comparative Example 3

Component (A) was first prepared in the manner of Application Example 2. Next, the diorganopolysiloxanes (e)-(h) used in Comparative Example 1 were added in the same manner as the diorganopolysiloxanes of Application Example 2. 100% cotton fabric, as above, was treated with these compositions. The hand, oil repellency and water repellency of the fabric after treatment were measured and the results are listed in Table IV.

**Table IV**

| | Hand | Oil Repellency | Water Repellency | Overall Evaluation |
|---|---|---|---|---|
| Application Example 2: diorganopolysiloxanes | | | | |
| (a) | A | 4 | 90-80 | Extremely Good |
| (b) | A | 4 | 90-80 | Extremely Good |
| (c) | A | 4 | 90-80 | Extremely Good |
| (d) | A-B | 4 | 80-90 | Extremely Good |
| Comparative Example 3: diorganopolysiloxanes | | | | |
| (e) | C-B | 4 | 80 | Somewhat Insufficient |
| (f) | C-D | 3 | 70-80 | Insufficient |
| (g) | C | 3 | 70-80 | Insufficient |
| (h) | D | 2 | 70 | No good |

## Claims

1. A fiber and textile treatment composition comprising:
(A) 100 parts by weight of vinyl polymer having perfluoroalkyl radicals with a carbon number of 5 or greater, and
(B) 5-50 parts by weight of organopolysiloxanes that have one or more epoxy-containing organic radicals, and one or more carboxyl groups represented by the formula:
-COOR⁶
wherein R⁶ is a monovalent radical selected from the group consisting of hydrogen atoms, hydrocarbon radicals, and silyl radicals represented by the formula:
-SiR₃
wherein each R is a radical independently selected from monovalent hydrocarbon radicals having 1-10 carbon atoms or radicals represented by the formula:
-R³-SiR₃₋ₐ(OR⁴)ₐ
wherein R is as above, R³ is selected from divalent hydrocarbon radicals or sulfur-containing divalent hydrocarbon radicals, R⁴ is selected from hydrogen atoms or monovalent hydrocarbon radicals, and a is an integer from 1 to 3.

2. The composition of Claim 1 further comprising said composition in an aqueous emulsion form.

3. The composition of Claim 1 or Claim 2 further comprising an organic solvent.

4. A method of treating a fiber or textile, comprising the steps of:
(I) immersing and soaking the fiber or textile in a composition according to any of Claims 1 to 3;
(II) squeezing said soaked fiber or textile until a squeezing ratio of 100% is obtained;
(III) drying the squeezed fiber or textile; and
(IV) heating the dried and squeezed fiber or textile to a temperature of 150°C.
